

(Specimens.)

R. ALEXANDER.

PROCESS OF REFINING CRUDE ASPHALTUM.

No. 435,198.

Patented Aug. 26, 1890.



Attest:  
Geo. T. Smallwood,  
M. M. Westover.

Inventor:  
Robert Alexander,  
By Kenne & Goldsborough,  
Attest.

# UNITED STATES PATENT OFFICE.

ROBERT ALEXANDER, OF JERSEY CITY, NEW JERSEY.

## PROCESS OF REFINING CRUDE ASPHALTUM.

SPECIFICATION forming part of Letters Patent No. 435,198, dated August 26, 1890.

Application filed January 8, 1890. Serial No. 336,283. (Specimens.)

*To all whom it may concern:*

Be it known that I, ROBERT ALEXANDER, a citizen of the United States, residing at Jersey City, in the county of Hudson and State of New Jersey, have invented certain new and useful Improvements in Refining Crude Asphaltum; and I do hereby declare the following to be a full, clear, and exact description of the invention, such as will enable others skilled in the art to which it appertains to make and use the same.

Prior to my invention it has been customary to effect the desiccation and liquefaction of native asphaltum (Trinidad and the like) by placing it in vessels prepared for the purpose and subjecting it therein to external heat during a period of four or five days, at a temperature ranging between 400° and 500° Fahrenheit. This long period of exposure to the comparatively high heat referred to has heretofore been found necessary in order to drive off completely the water present in the native material and to fully melt said material or bring it to a homogeneous liquid condition. In many instances, however, it has been found impossible, even at the end of four or five days, to entirely liquefy the mass of crude material. The central portion of the charge, being relatively distant from the heated walls of the containing-vessel, does not always receive a sufficient amount of heat to be melted, and frequently remains as an un-reduced core after the outer portions are desiccated and liquefied. Under such circumstances it is impracticable to raise the furnace heat so as to reduce the said core, for the reason that the higher heat that would be necessary for that purpose would burn or destructively distill the material already melted. It has therefore been found necessary in these instances to interrupt the operation and tap off the melted portion, the un-reduced core remaining in the containing-vessel and the space around it being thereupon filled in with fresh material for a subsequent melting. It is manifest that when this un-reduced core is present the effective melting capacity of the vessel is materially diminished and the product of the operation proportionally decreased.

One of the objects of my invention is to

more uniformly distribute the heat throughout the charge during the entire operation, thereby lessening its duration and preventing the formation of a core.

The treatment to which the desiccated product has been subjected has deprived it in great measure of the asphaltum oils originally contained in the crude material, said oils having been largely driven and dissipated or destructively distilled by the high heat employed.

In order to impart plastic properties to the product, so as to render it suitable for pavements and the like, it has been customary to add to it from eighteen to twenty per cent. of crude petroleum. This percentage of crude petroleum is added when the desiccated material is in a melted condition, and the melting-temperature is maintained until the most intimate admixture of the two is secured, the crude petroleum serving as a solvent or diluent. Experience has shown, however, that the addition of this crude petroleum causes the desiccated material when laid as a pavement to begin to disintegrate or rot within a comparatively short time. I have discovered that this disintegration is due to the presence of the crude petroleum and to the absence of the asphaltum oils driven off during the melting operation, and is diminished in proportion as the original percentage of those oils is restored to the desiccated material, of which they form the material and appropriate solvent. I have accordingly adopted means for recovering the greater portion of said oils during the melting operation as condensable by-products of the manufacture, for the purpose of returning them thereafter to the desiccated material, so as to diminish or entirely supplant the crude petroleum. In order, however, to retain as many of the said oils as possible in the desiccated material during the operation, and in order to prevent material destructive distillation of the remainder, I employ a procedure enabling me to conduct the desiccation and liquefaction at a comparatively low temperature, so that those oils only which are volatile at or below such temperature shall be given off to the condenser.

The entire volatile products, consisting of watery vapors, asphaltum-oil vapors, small

quantities of tar and soot, and such light uncondensable gases as are inseparable from the operation, are received in an appropriate condensing and separating vessel, whence the 5 condensable matters pass to a convenient receptacle, while the combustible gases are led into the fire-place and burned therein. As a consequence, the operation is quite devoid of noxious or deleterious matters prejudicial to 10 public health or comfort and may be practiced without restriction from local authorities.

In the accompanying drawings, Figure 1 represents in vertical section and partial elevation a form of apparatus appropriate to my 15 invention, and Fig. 2 represents a like view, on an enlarged scale, of certain details thereof.

Similar numerals of reference indicate similar parts in both figures.

20 Referring to the drawings, 3 indicates a suitable furnace provided with the usual adjuncts for supplying and maintaining an effective heat therein. Upon the fire-arches, as shown, rests the melting or desiccating vessel, consisting, 25 preferably, of the lower cylindrical portion 4 and the hood or cap 5, adapted to be firmly and securely bolted thereto. Danger of explosion is prevented by means of the safety-valve device 6, mounted upon the short pipe 30 7, connected to the top plate of the hood 5 and communicating freely with the interior of the desiccating-vessel. A pipe 8 communicates with the pipe 7, and is also connected by means of the joint-coupling 9 with the 35 descending pipe 10, leading to the condenser and separator 11. The joint-coupling 9 is provided with a suitable screw-down valve 12, whereby the outer or proximate end of the pipe 8 may be closed when desired. The condenser and separator 11 is of a familiar type, 40 consisting of a main body portion, a curved entrance branch 13, and an upwardly-extended pipe 14, forming a continuation of the pipe 15. A glass gage 16 indicates the height 45 of liquid within condenser, and a draw-off pipe 17, having a stop-cock 18, serves to conduct the liquid condensates to the discharge 19, opening into the receptacle 20. The pipe 15 communicates by a stop-cock coupling 21 50 with the pipe 19 and with the gas-discharge pipe 22, opening into the furnace. Air under pressure is supplied to the desiccating-vessel by means of the pipe 23, having the screw-down valve 24. The pipe 23 extends inwardly 55 to the center of the vessel and then downwardly by the descending pipe 25 to the lower part thereof, where it communicates with horizontal branch pipes 26, provided with a series of bottom perforations, as shown.

60 The operation of the invention is as follows: The crude or native Trinidad or other asphalt is thrown in lumps in the usual manner into the desiccating-vessel and closely envelops the central pipe 24. The heat from 65 the furnace is communicated at once to the bottom of the vessel 4 and by conduction to the sides of said vessel and to its contents,

which gradually rise in temperature. The valves 24 and 12 being opened, a current of air under pressure enters through the pipe 23, 70 and passing downwardly through the pipe 24 to the branches 26 passes out through the openings therein. On escaping through the openings and at the hottest portion of the desiccating-vessel the condensed air immediately expands and passes upward in streams through the superjacent material, giving up its heat thereto and causing the material to give up at first a large amount of watery vapor, which issues, together with the air, 80 through the pipes 8 10 into the condenser and separator 11. With the watery vapor are also carried off some of the lighter asphaltum oils, partly in the form of condensable vapors and partly as uncondensable gases. The latter pass through the pipes 14, 15, and 22 into the furnace-space, where they are consumed. The watery vapor and oily vapors are condensed and pass by the pipes 17 and 19 to the common receptacle 20, where they separate by gravity, the oil floating on the top of the water. The operation thus begun is continued until watery vapor is no longer given off from the desiccating-vessel and until the charge is completely melted. As the charge 90 melts, the liquefied portion cores or submerges the branch pipes 26, and the air as it escapes bubbles up with expansive energy through the liquid, maintaining it in vigorous agitation. The unrestrained constant 95 circulation thus induced disseminates the heat with great uniformity throughout the mass and enables me to employ a low temperature of from 250° to 300° Fahrenheit to effect the entire desiccation and at the same 100 time to complete the operation in a much shorter period of time than with the higher heats heretofore employed. The heat conductivity of the pipe 25 is also an important factor in shortening the time of treatment, 105 for the reason that it melts the asphaltum immediately contiguous to its walls, thereby permitting the heated air to rise in increased volume through the center of the charge and preventing the formation of a core. By the 110 aid of a suitable pyrometer care must be taken to maintain the temperature in the desiccating-vessel at the low minimum indicated. In practice I have found that a 115 temperature of 250° Fahrenheit sufficed for the complete elimination of the watery vapor and the full melting of the charge. This temperature is ordinarily maintained for about two days and a half, during which 120 period a considerable quantity of asphaltum-oil is obtained. At the end of said period this oil is restored to the purified asphaltum, either in complete substitution for the crude petroleum ordinarily employed or in partial substitution therefor should an insufficient quantity of the asphaltum oil be 125 available. I have found by experiment that the solvent power of the asphaltum oil for the purified asphalt is far superior to that 130

of the crude petroleum, in some instances amounting to three times that of the latter. It is therefore only necessary to employ a correspondingly small amount of the asphaltum oil in the final step of the process. After the addition of the asphaltum oil as a partial or entire substitute for the crude petroleum ordinarily employed, the operation is continued, as before, during a period of about twelve hours, but preferably at the higher temperature of 300° Fahrenheit, whereupon the desired product is obtained. It will be understood that before adding the asphaltum oil in this last stage of the operation I preferably separate from it, by filtration, deposition, or otherwise, any objectionable foreign matters that may be present in it, such as soot, tar, water, or the like.

Having thus described my invention, what I claim is—

1. The process of refining crude asphaltum and obtaining an improved product therefrom, which consists in desiccating the crude asphaltum at a low temperature, recovering the condensable oils given off during desiccation, and subsequently returning said oils to the desiccated material, substantially as described.

2. The process of refining crude asphaltum, which consists in simultaneously desiccating and melting the same by subjecting it to heat until melted and simultaneously removing the water by passing through the charge a

current of air during the melting operation, substantially as described. 35

3. The process of refining crude asphaltum, which consists in subjecting the same to a temperature of from 250° to 300° Fahrenheit and simultaneously passing through it a current of air, said air being admitted at or near 40 the bottom or hottest portion of the charge, whereby it is suddenly expanded, substantially as described.

4. As a new composition of matter, desiccated asphaltum containing in solution the 45 condensable asphaltum oils given off during desiccation, substantially as described.

5. In the refining of crude asphaltum, the process of preventing the formation of an unreduced central core within the refining- 50 vessel, which consists in admitting air at or near the bottom of the charge and locating a portion of the air-inlet pipe within the center of the charge, whereby the charge surrounding said pipe is melted by conduction 55 therefrom, thereby facilitating the passage of the air upward through the said central portion, so as to rapidly liquefy it, substantially as described.

In testimony whereof I affix my signature in 60 presence of two witnesses.

ROBERT ALEXANDER.

Witnesses:

D. G. STUART,  
JOHN C. PENNIE.